

## UNITED STATES PATENT OFFICE

2,618,599

HIGH MELTING POINT CALCIUM GREASE  
OF LOW SOAP CONTENT

Laurence F. King, Sarnia, Ontario, and Warren C. Pattenden, Courttright, Ontario, Canada, assignors to Standard Oil Development Company, a corporation of Delaware

No Drawing. Application June 1, 1951,  
Serial No. 229,548

10 Claims. (Cl. 252—40.5)

1

The present invention relates to high melting point calcium greases of low soap content. It relates particularly to lubricating greases composed substantially of mineral base lubricating oils thickened to a grease consistency with a combination of thickeners which impart better properties to the grease than have commonly been obtained in prior art compositions.

Conventional calcium base greases are widely used because of their smooth texture and their structural stability at normal temperatures. They are relatively easy to manufacture. For service at temperatures which do not exceed about 200° F. the conventional calcium base lubricating greases are quite satisfactory lubricants. They are relatively inexpensive because their principal ingredients are cheap. They have one well known deficiency, however, in that they commonly require the presence of a small amount of water to maintain stability and they cannot be used at temperatures high enough to drive out this water. If conventional calcium base greases are heated to a temperature substantially equal to or in the neighborhood of the boiling point of water, or higher, the water which they contain, which is a structure stabilizer, is evaporated and the calcium soap separates readily from the oil with resulting failure of lubrication.

It has been found in the prior art that the dropping point of conventional calcium greases can be substantially raised by the addition of low molecular weight fatty acids to the usual higher fatty materials. Upon saponification of the higher fatty materials, the lower acids are converted into salts at the same time that the soap is formed. Thus, it has been suggested in the prior art that the addition of lower acids such as acetic acid, lactic acid, and various other low molecular weight acids tends to improve the dropping point of calcium greases. Apparently these acids, when co-neutralized with the high molecular weight fatty materials, form salts with the metal base which salts in turn form a complex with the soaps. In particular it has been found possible in the prior art to prepare high melting calcium greases by saponifying with the lime mixtures of stearic acid and lactic acid, or by saponifying mixtures of 12-hydroxy stearic acid and lactic acid.

Greases prepared as just described, however, have one notable deficiency. They require a relatively large amount of the salt and soap for thickening the lubricating oil to a reasonably firm grease consistency. As will be seen in the table, below, greases of only moderate consistency made with the ingredients just mentioned may require as much as 21 to 31.5% of the combined soap and salt. Since the soap constituents are usually much more costly than the lubricating oil used, the use of such high proportions

of thickener is expensive and therefore objectionable. Also, the high soap content makes the grease abnormally viscous at room temperatures. The harder or more viscous greases are undesirable for many purposes because, for example, they are difficult to dispense in commercial grease dispensing equipment.

The present invention is based on the discovery that greases of the general type just described can be greatly improved by replacing a part of the usual fatty acid (stearic or hydroxy stearic acid) by a partially dehydrated castor oil or fatty acid derived therefrom before saponifying with lime. Thus, a grease containing a combination of three thickening agents, namely, the calcium soap of stearic or hydroxy stearic acid, or of equivalent substantially saturated fatty acids having between 12 and 22 carbon atoms per molecule, the calcium soap of a partially dehydrated castor oil, and the calcium salt of a low molecular weight carboxylic aliphatic acid makes a superior product.

The partially dehydrated castor oil is preferably dehydrated by known processes until its iodine number has been increased from a normal 84, or so, to about 90 to 110. Complete dehydration of castor oil raises the iodine number to as high a value as 118 to 140. Complete dehydration is useful for the preparation of synthetic drying oils, but for the purposes of the present invention, it is desirable that dehydration be carried out only partially to the extent indicated by an iodine value of 90 to 110, and preferably between about 95 and 105.

As is well known in the art, castor oil can be dehydrated by heating with sulfuric acid or phosphoric acid, or with sodium acid sulfate to carry out the dehydration to the desired extent.

The low molecular weight acid is preferably a hydroxy aliphatic acid having not more than 6 carbon atoms, for example, 3 to 6 carbon atoms. Specifically preferred acids are lactic acid, or hydrylic acid, but any of the hydroxy butyric acids can also be used.

Preferably the three soap-forming or salt-forming acidic materials, namely the high molecular weight fatty acid, or natural fat, the partially dehydrated castor oil, and the low molecular weight carboxylic acid are used in roughly equal proportions by weight prior to saponification. The invention contemplates, however, the use of as little as 1% and as much as 10% by weight based on the total grease composition of each of the three soap or salt ingredients which form the thickener. The specifically preferred compositions consist essentially of about 85 to 93% by weight of lubricating oil, 2 to 5% of the calcium soap of stearic or hydroxy stearic acid, 12-hydroxy stearic acid being specifically preferred, 2 to 5% of the calcium soap of the par-

tially dehydrated castor oil, and about 2 to 5% of the calcium salt of the low molecular weight acid, for example, lactic or hydrylic acid. Minor amounts of conventional additives which do not greatly affect the grease structure may be included if desired.

Grease compositions made according to the general formulas just described may be prepared by conventional methods. The soap-forming and salt-forming fats and acids are mixed with a portion of the lubricating oil, and the calcium hydroxide is added for saponification. The balance of the lubricating oil is added thereafter or while the reaction takes place. Greases prepared in this manner have unusually high dropping points for calcium greases, usually between 350 and 450° F. Their resistance to shear, as determined in the standard ASTM grease worker, is very good. In particular, they show excellent resistance against oil bleeding at high temperatures.

It is interesting to note that the calcium soap of the partially dehydrated castor oil by itself is insoluble in mineral oil. Furthermore, it is not dispersible in mineral lubricating oil at normal grease making temperatures. In the presence of calcium stearate, or hydroxy stearate and calcium lactate, however, the soap of the treated castor oil may be readily dispersed at a temperature of 400 to 425° F. The very lack of solubility of this soap appears to be advantageous and is probably responsible for the marked increase in yield, that is, the superior consistency obtained with a given amount of thickener.

The preparation of calcium greases which show bleeding of less than 3% of their weight at temperatures of 225° F. for a product of low soap content is considered an important improvement in the art. Several samples of grease were made with various quantities of the complex thickener and with variations in other ingredients. Generally speaking these greases showed low bleeding after 100 hours at 225° F. in a 28 mesh cone. These greases also showed good resistance against water, 55% of the grease being retained in a single row ball bearing revolved at 800 to 900 R. P. M. and immersed in water for one-half hour at 150° F. The retention of 55% of the grease in the bearing under these conditions appears to be outstanding. The grease, furthermore, stood up well in a standard wheel bearing test, operating at a temperature of 220° F. Conventional calcium greases are quickly dehydrated

and the oil separates from the soap in a very short time at such a temperature.

While various low molecular weight acids may be employed a conventional lactic acid of "Food Process Grade," sold as an 80% concentration in water, has proved to be very satisfactory in practice.

The partially dehydrated castor oil which is presently preferred is a castor oil that has been dehydrated to the extent of removing approximately one-half of the hydroxyl groups by a suitable treatment. The castor oil may be heated in the presence of a catalyst such as lead oxide to carry out the partial dehydration. A more drastic heat treatment is likely to yield a completely dehydrated castor oil which is not a desirable ingredient because of its excessive drying tendencies.

Six experimental greases were prepared to determine their relative properties and characteristics. Example I is a conventional stearic acid-lactic acid lime base grease containing about 21% of the soap-salt complex thickener in mineral base lubricating oil. Example II contained about 31.5% of a combination of the calcium soaps of 12-hydroxy stearic acid and lactic acid. Examples III, IV, V and VI include the ingredients of the present invention; Example V substitutes hydrylic acid for lactic acid.

The dispersion of the soap and salt may be facilitated by the addition of a small amount, for example 0.5 or 1% to 5%, based on the weight of the total grease composition, of a high molecular weight alcohol such as hydroabietyl alcohol. This is an optional material, however, and need not always be used. Conventional oxidation inhibitors such as phenyl alpha naphthylamine, or the corresponding beta product may be used in the usual quantities, for example 0.1 to 1%, preferably about 0.5%. Other inhibitors, metal deactivators, etc., may be used in usual proportions, where needed.

Although the invention has been described in connection with the production of greases based on mineral oil as the lubricant, it is equally applicable to the production of greases using synthetic oils. Care must be taken, however, in the preparation of the soap, to avoid hydrolysis or other decomposition of the synthetic oil. It is preferred to form the soap in mineral oil and later to add synthetic oils such as dibasic acid esters, related complex esters, poly glycols, poly glycol ethers, and the like as is well known in the art.

The data are summarized in the table.

Table

| Example                                                      | I     | II   | III       | IV   | V         | VI   |
|--------------------------------------------------------------|-------|------|-----------|------|-----------|------|
| Ingredients, percent by wt.:                                 |       |      |           |      |           |      |
| Stearic Acid.....                                            | 13.6  | 0    | 0         | 3.55 | 3.7       | 0    |
| 12-hydroxy Stearic Acid.....                                 | 0     | 20.0 | 2.4       | 0    | 0         | 3.1  |
| Partially Dehydrated Castor Oil.....                         | 0     | 0    | 2.4       | 3.55 | 3.7       | 3.1  |
| Lactic Acid (80% Conc.).....                                 | 6.8   | 10.0 | 2.4       | 3.55 | 0         | 0    |
| Hydrylic Acid <sup>1</sup> .....                             | 0     | 0    | 0         | 0    | 4.0       | 0    |
| Hydroabietyl Alcohol.....                                    | 2.75  | 4.0  | 0.8       | 0    | 0         | 1.0  |
| Lime.....                                                    | 5.4   | 7.8  | 1.95      | 3.05 | 3.2       | 2.2  |
| Phenyl Alpha Naphthylamine.....                              | 0.5   | 0.5  | 0.5       | 0.5  | 0         | 0.5  |
| Mineral Oil 320, <sup>2</sup> 45 V. I.....                   | 70.95 | 57.7 | 89.55     | 0    | 0         | 0    |
| Mineral Oil 150, <sup>2</sup> 85 V. I.....                   | 0     | 0    | 0         | 85.8 | 85.4      | 0    |
| Mineral Oil 150, <sup>2</sup> 45 V. I.....                   | 0     | 0    | 0         | 0    | 0         | 87.0 |
| Inspections:                                                 |       |      |           |      |           |      |
| Worked Penetration ASTM.....                                 | 265   | 260  | 290       | 285  | 255       | 325  |
| Stability (Pen. 10,000 Strokes <sup>3</sup> ).....           | 250   | 320  | (no data) | 290  | (no data) | 350  |
| Percent Bleeding, 100 hrs. @ 225° F.<br>in 28 mesh Cone..... | Nil   | 4.8  | (no data) | 0.6  | (no data) | 2.9  |
| ASTM Dropping Point, ° F.....                                | 450+  | 425+ | 390       | 448  | (no data) | 350  |
| Total Thickener, percent by wt. (Soap<br>and Salt).....      | 21.1  | 31.5 | 7.5       | 11.0 | 11.9      | 9.7  |

<sup>1</sup> Prepared by hydrolysis of beta-propiolactone at room temperature.

<sup>2</sup> S. S. U. @ 100° F.

<sup>3</sup> At 2,500 Sec.<sup>-1</sup> rate of shear in ASTM grease worker.

It will be understood that various conventional additives such as anti-oxidants, extreme pressure compounds, thickener agents, viscosity index improvers, and the like may be incorporated in grease compositions made according to the present invention. In general the lubricating oils preferred are of mineral base with a viscosity between 100 and 5000 S. S. U. at 100° F. and they may be of various viscosity indexes. The higher viscosity index oil, for example of 85 V. I. or higher is particularly useful for service at widely varying temperatures with the combination of soaps and salts described herein. By the present invention, difficulties commonly encountered in using high V. I. oils (because of their traditional incompatibility with soaps) are largely eliminated.

What is claimed is:

1. A lubricating grease composition comprising 70 to 95% by weight of a lubricating oil thickened to a grease consistency with 1 to 10% by weight, based on the total composition, of calcium soap of substantially saturated fatty material of the C<sub>12</sub> to C<sub>22</sub> range, 1 to 10% of calcium soap of partially dehydrated castor oil, and 1 to 10% of the calcium salt of an aliphatic hydroxy carboxylic acid having not more than 6 carbon atoms per molecule.

2. Composition according to claim 1 wherein said lubricating oil is a mineral base oil.

3. Composition according to claim 1 wherein said substantially saturated fatty material is stearic acid.

4. Composition according to claim 1 wherein said substantially saturated fatty material is predominantly 12-hydroxy stearic acid.

5. A lubricating grease composition consisting essentially of 70 to 95% by weight of mineral base oil of 100 to 5000 S. S. U. viscosity at 100° F., 1 to 10% of calcium soap of at least one fatty acid selected from the group which consists of

stearic acid and hydroxy stearic acid, 1 to 10% of calcium soap of partially dehydrated castor oil having an iodine number between about 90 and 110, and 1 to 10% of the calcium soap of a hydroxy aliphatic carboxylic acid having not more than 6 carbon atoms.

6. A composition according to claim 5 wherein said fatty acid is predominantly 12-hydroxy stearic acid.

7. A composition according to claim 5 wherein said fatty acid is predominantly stearic acid.

8. A lubricating grease composition having essentially the formula by weight:

85 to 94% mineral lubricating oil  
2 to 5% calcium soap of 12-hydroxy stearic acid  
2 to 5% calcium soap of partially dehydrated castor oil

2 to 5% of the calcium salt of lactic acid

9. A lubricating grease composition having essentially the formula by weight:

85 to 94% mineral lubricating oil  
2 to 5% calcium soap of 12-hydroxy stearic acid  
2 to 5% calcium soap of partially dehydrated castor oil  
2 to 5% of the calcium salt of hydrylic acid

10. Composition according to claim 8 to which is added 0.5 to 5% of hydroabietyl alcohol.

LAURENCE F. KING.  
WARREN C. PATTENDEN.

#### REFERENCES CITED

The following references are of record in the 35 file of this patent:

#### UNITED STATES PATENTS

|    | Number    | Name           | Date           |
|----|-----------|----------------|----------------|
| 40 | 2,197,263 | Carmichael     | Apr. 16, 1940  |
|    | 2,417,429 | McLennan       | Mar. 18, 1947  |
|    | 2,450,219 | Ashburn et al. | Sept. 28, 1948 |